# EUROPEAN PATENT SPECIFICATION

(11) **EP 0 002 335 B1**
(45) Date of publication and mention of the grant of the patent: **10.06.1981**
(21) Application number: 78300660.4
(22) Date of filing: 23.11.1978
(51) Int. Cl.: C22C 19/07, H01F 1/04, H01H 1/02

(54) **Semi-hard magnetic material for a reed switch reed piece, process for producing the reed piece and use thereof**
Halbhartes magnetisches Material für ein Kontaktstück für einen Reed-Schalter sowie Verfahren zur Herstellung des Kontaktstückes und seine Verwendung
Matériau magnétique semi-dur pour contact d'un interrupteur du type Reed, procédé de fabrication d'un tel contact et son utilisation

(30) Priority: 29.11.1977 JP 142157/77
(43) Date of publication of application: 13.06.1979
(73) Proprietor: FUJITSU LIMITED, Kawasaki-shi, Kanagawa 211 (JP)
(72) Inventor: Suzuki, Yuichi, Zushi-shi Kanagawa-ken (JP); Okada, Masanori, Yokohama-shi Kanagawa-ken (JP); Henmi, Zenzo, Kawasaki-shi Kanagawa-ken (JP)
(74) Representative: Jennings, Roy Alfred

## Description

The present invention relates to semi-hard magnetic materials, which are suited for reed pieces of a self-holding type reed switch, a process for producing a reed piece from the semi-hard magnetic materials and a use of the reed piece so produced. Such materials should possess a hysteresis loop shape and residual magnetization property suited for application in a self-holding type reed switch. Specifically the semi-hard magnetic materials utilized in a reed piece of a reed switch should preferably possess the following properties.
1. Both saturated magnetic flux density (Bs) and residual magnetic flux density (Br) are high.
2. The square hysteresis loop exhibits a high squareness ratio (Br/Bs) and a high "fullness factor". The term "fullness factor" used herein is represented by the formula: wherein (BH)max is the maximum magnetic energy product and Hc is coercive force.
3. The coercive force (Hc) is usually in the range between 10 to 50 Oe. The coercive force should be more than 50 Oe for application of the semi-hard magnetic materials to reed switches where mutual demagnetization, explained hereinafter, is severe.
4. Plastic workability is excellent, i.e. these materials are capable of being easily cold worked into any desired shape or size such as, for example, a fine wire rod having a diameter as small as less than 1 mm.
5. The plating or soldering property is excellent, i.e. a surface layer of the semi-hard magnetic materials used for forming a reed piece can be reliably produced by the plating-or soldering-process.
6. When the semi-hard magnetic materials are exposed to a high temperature at the time of sealing the reed pieces having the above mentioned surface layer in a glass capsule of the reed switch, the magnetic properties of the reed pieces are not deteriorated by the increase of temperature.

When the reed switches are used in a four-wire crosspoint switch matrix of an electronic switching system, mutual demagnetization occurs between the four reed switches. As a result of the demagnetization, the coercive force and the squareness ratio of the semi-hard magnetic materials must be higher than in the reed-switches used in a two-wire crosspoint switch of an electronic switching system.

In U.S Patent No. 3,989,557, filed by the present Applicant, there is described a process for producing semi-hard magnetic material, wherein an alloy material comprising from 73 to 93% of cobalt, from 1 to 5% of niobium and iron in balance is subjected to (1) a process annealing at a temperature of 900° or higher, and subsequently, (2) a final cold working at a reduction of area of 75% or higher. The same U.S. patent also describes a process for producing a semi-hard magnetic material, wherein the alloy material, which is cold worked as stated above, is further subjected to ageing at a temperature of 950°C and higher. The semi-hard magnetic material, in the U.S. Patent mentioned above, however, is disadvantageous in the fact that the cold working property thereof is deteriorated by the increase of the niobium content in the range of from 1 to 5%, although the coercive force of the semi-hard material is increased by such increase of niobium. In addition, deterioration of cold-workability is particularly remarkable when an attempt is made to increase niobium to more than 5%.

The alloy material of the U.S. Patent mentioned above may contain, for example, tantalum, titanium, vanadium, zirconium, molybdenum, chromium, tungsten and the like. The amount of these metals used in addition to niobium is usually such that the ratio by weight of these metals to niobium is below 30/70. These metals form intermetallic compounds in the same a manner as niobium forms the intermetallic compounds, according to the description of U.S. Patent No. 3,989,557.

The present Application proposed in the U.S. Patent No. 3,983,916 an improved process for removing the deterioration of the cold workability, wherein an alloy material consisting essentially of from 73 to 93% of cobalt, from 3 to 7% of niobium and iron in balance is subjected to (1) a solution treatment, i.e. a heating at a temperature of 1000°C or higher followed by a rapid cooling through at least the temperature range between 800°C and 500°C, then, (2) a cold working at a reduction area of 75% or more, and subsequently, (3) an ageing at a temperature in the range from 500 to 900°C. The present Inventors investigated further in detail the improved process mentioned above and realized that this process involves the following problem, although the cold workability of the semi-hard magnetic material is in fact enhanced to some extent by the improved process. Unless the bar or wire of the semi-hard magnetic material is carefully drawn in the cold drawing process the bar or wire is liable to rupture. Second, the cold workability of the semi-hard magnetic material is seriously degraded, to such an extent that the cold working cannot be practiced industrially, when an attempt is made to provide the material with a coercive force higher than 40 Oe. In the semi-hard magnetic material mentioned above and containing 3 to 7% of niobium, the Nb content and Fe content must be increased to 5% or higher and 18% or higher, respectively, with the result that the coercive force is increased more than 40 Oe, but the cold workability is deteriorated. It is, therefore, practically impossible to obtain from the Co-Fe-Nb alloy material, a semi-hard magnetic material having a coercive force of from 40 to 70 Oe and which is suited for the reed switches to be mounted in a four-wire crosspoint switch matrix of an electronic switching system.

British Patent No. 1,118,466 discloses a method of producing a ferromagnetic body of an alloy comprising cobalt and iron in a weight ratio of from 85:15 to 95:4.5 together with a small amount of vanadium, molybdenum, niobium, chromium, titanium, tantalum and/or tungsten in a total amount of not more than 6% byt weight. The alloy is annealed and then cold worked. The cold working produces the desired hysteresis characteristics. With this alloy, the highest coercive force is obtained with a minimum iron content. There is a tendency for this alloy to be very brittle and this tendency is only partly overcome by the annealment before cold working.

A semi-hard magnetic material having a high coercive force is available under the name of VACOZET 655, which is sold by the VACUUMSCHMELZE Company, in Federal Republic of Germany. This semi-hard magnetic material comprises 30% iron 10.6% nickel, 1.2% aluminium, 2.4% titanium and cobalt in balance. Since the magnetic properties of this semi-hard magnetic material are unstable, with the result that, for example, the coercive force is reduced by heat, the material is not suitable for reed pieces, which are sealed or enclosed in a glass capsule of a reed switch, In addition, since the semi-hard magnetic material of VACOZET 655 includes aluminium as well as titanium, the plating and soldering properties of the material are not superior to those of the Co-Fe-Nb alloy.

It is an object of the present invention to improve a semi-hard magnetic material for reed pieces of a reed switch containing mainly cobalt, and additionally iron and niobium, as well as one additive element which can form an intermetallic compound, so that the cold workability is not deteriorated with an enhancement of the coercive force.

It is further object of the present invention to provide a semi-hard magnetic material suited for the reed pieces of reed switches, which are mounted in each crosspoint of the four wire type crosspoint in an electronic exchange system.

It is also an object of the present invention to prevent the rupture of the reed pieces during the cold working of the reed pieces of a reed switch and to enhance the coercive force of the produced reed pieces.

In accordance with the present invention, there is provided a magnetic material for a reed piece of a reed switch, said material containing (a) cobalt and iron, which forms a matrix of said material having a face centred cubic lattice, (b) additionally niobium, which niobium is precipitated in said matrix as intermetallic compounds and provides said material with the required coercive force, and (c) one element, which is added in a predetermined amount, characterised in that said one element is molybdenum and is present in said material in an amount of not less than 2% by weight so that said matrix is composed of said face centred cubic lattice and a body centred cubic lattice, said material has a coercive force of not less. than 35 Oe, preferably from 40 to 70 Oe, more preferably from 60 to 70 Oe, and the components of said material are present in the following ranges by weight:
iron from 12 to 18%, preferably from 15 to 18%;
niobium from 2 to 4%;
molybdenum from 2 to 5%;

and the balance essentially cobalt, thereby providing said material with a residual magnetization flux density of not less than 11 kG, preferably 13 kG, and a fullness factor as defined above, of not less than approximately 0.80.

The present invention also consists, according to another of its aspects in a process for producing a reed piece of a reed switch from a magnetic material containing a major proportion of cobalt and iron, and additionally niobium and one element which is added in a predetermined amount, the process comprising the steps of solution-treating said material, cold working said solution-treated material at a predetermined reduction area, ageing said cold worked material, and enclosing said aged material in a glass capsule of said reed switch, characterised in that molybdenum is selected as said one element in an amount of from 2 to 5% by weight and the iron content is adjusted to an amount in the range of from 12 to 18%, preferably from 15 to 18%, by weight, and the niobium content in an amount in the range of from 2 to 4% by weight, said cold working is performed at a reduction of area of at least 90%, and, due to said molybdenum selection, (a) maintaining the hardness of said cold worked material at a value not exceeding 450 Vickers Pyramid Number, (b) preventing the decomposition of the cobalt matrix phases of the face centred cubic lattice into two different kinds of phases during said cold working, and (c) preventing the rupture of said material during said cold working; said cold worked material is aged at a temperature of from 600 to 750°C, preferably from 650 to 700°C, thereby decomposing said cobalt matrix phases into (a) the phases of intermetallic compounds precipitated in the matrix of said aged material, (b) the original matrix phases of said face centred cubic lattice and (c) the new matrix phases of a body centred cubic lattice; and the semi-hard magnetic alloy is provided with a coercive force not less than 35 Oe, preferably from 40 to 70 Oe, more preferably from 60 to 70 Oe, a residual magnetisation flux density of not less than 11 kG, preferably 13 kG, and a fullness factor as defined above, of not less than approximately 0.80.

The basic component of the semi-hard magnetic material according to the present invention is cobalt, which is contained therein in an amount of from 73 to 84%, preferably from 75 to 81 %. When the cobalt content is less than 73%, the alloy material is so hard that the workability thereof is deteriorated. As a result, both the squareness ratio and the fullness factor of the semi-hard magnetic material is disadvantageously reduced.

The alloy material according to the present invention exhibits at the solution treated state a face centred cubic lattice, because this alloy material mainly contains cobalt and iron. However, when the cobalt content is less than 72%, a part of the alloy material crystals having the face centred cubic lattice is transformed into a body centred cubic lattice during the cold working, with the result that the plastic workability of the cobalt based alloy material is reduced. If the cobalt content exceeds 84%, the workability of the alloy material is also reduced. This is because a part of the alloy material crystals having the face centred cubic lattice is transformed into a hexagonal close packed lattice, with the result that the plastic workability of the cobalt based alloy material is reduced. In addition, if the cobalt content exceeds 84%, the contents of molybdenum, iron and niobium are relatively reduced, and thus, the magnetic properties of the semi-hard magnetic materials are disadvantageously degraded.

The niobium provides, in combination with molybdenum, the semi-hard magnetic material with the required coercive force. When the niobium content is less than 2%, the coercive force is too low. On the other hand, when the niobium content exceeds 4%, the workability of the cobalt based alloy material is degraded. With an increase of the niobium content, intermetallic compounds containing niobium tend not to be dissolved, and thus, remain in the cobalt matrix after the solution treatment of the cobalt based alloy material.

The iron provides the semi-hard magnetic material with the required coercive force, saturation flux density and residual magnetization. When the iron content is less than 12%, the coercive force, saturation flux density and residual magnetization are too low. When the iron content exceeds 18%, the cold workability of the cobalt based alloy material is reduced. The iron content is therefore from 12 to 18%.

If the semi-hard magnetic material consists only of cobalt, iron and niobium, the cold workability thereof is deteriorated when an attempt is made to increase the coercive force thereof by adjusting the niobium content. The feature of molybdenum resides in the fact that the coercive force is enhanced but the cold workability is not deteriorated substantially. The molybdenum content of 2% or more is essential for sharply increasing the coercive force. When the molybdenum content exceeds 5%, the residual magnetization is however, lowered.

The process for producing the semi-hard magnetic material according to the present invention includes the conventional steps of melting the raw materials for obtaining the alloy material, casting the melt into an ingot, hot- working the ingot, solution-treating the hot- worked alloy material, cold working, and subsequently ageing the alloy material. In the melting step, the conventional raw materials, such as an electrolytic cobalt, an electrolytic iron, a ferromolybdenum metal and a ferro- niobium metal, are melted in a high frequency, induction furnace, preferably in a vacuum, high frequency, induction furnace. The obtained melt is cast into a mold to produce an ingot, and the ingot is subjected to a homogenizing annealing. The ingot is then worked by a hot swaging machine, a cold swaging machine and a cold drawing machine, thereby producing a wire, a tape or a small bar. Any conventional process for producing the wire etc., can be employed in producing the semi-finished product of semi-hard magnetic material.

The semi-finished product mentioned above is heated at a temperature of from 1050 to 1200°C, preferably from 1050 to 1150°C, and should subsequently be rapidly cooled. The semi-finished product may then be subjected to a peeling by the dies, if necessary.

The semi-hard magnetic material according to the present invention, which consists of the Co-Fe-Nb-Mo alloy, can be used for the reed pieces of a reed switch, on which pieces a surface coating, for example a rhodium plating, must be applied. Since this semi-hard magnetic material contains neither titanium or aluminium, the surface coating is uniform and exhibits a high adhesive strength.

The present invention is explained in detail hereinafter with reference to the drawings, wherein:
Fig. 1 is a graph indicating the change of resistivity upon an ageing temperature of a Co-15%Fe-4%Nb-xMo alloy materials;
Fig. 2 is a graph indicating the relationship of the hardness after drawing with regard to the contents of additional elements added to several cobalt-based alloys;
Fig. 3 is a graph indicating the relationship of the hardness after drawing with regard to the coercive force of two cobalt-based alloys;
Fig. 4 is a general view of a four wire crosspoint switch;
Fig. 5 is a partially enlarged view of Fig. 1;
Fig. 6 is a crosspoint, in which the semi-hard magnetic material according to the present invention is used;
Figs. 7A, B and C are graphs indicating the change of the coercive force, the residual flux density and the squareness ratio, respectively, as a function of the aging temperature of Co-15%Fe-4%Nb-x%Mo allovs;
Figs. 8A and B are graphs indicating the change in residual flux density and coercive force, respectively, of the alloy materials of Fig. 7, as a function of the molybdenum content of the alloy;
Figs. 9A, B and C are graphs with regard to Co-18%Fe-3%Nb-x%Mo alloys similar to Figs. 7A, B and C, respectively;
Figs. 10A and B are graphs with regard to the Co-18%Fe-3°/Nb-x%Mo alloys, similar to Figs. 8A and B, respectively;
Figs. 11A, B and C are graphs with regard to Co-x%Fe-4%Nb-3%Mo alloys, similar to Figs. 7A, B and C, respectively; and
Figs. 12A and B are graphs indicating the changes in residual flux density and coerceive force, respectively, of the alloy materials of Fig. 11, with regard to the iron content of these alloy materials.

The semi-hard magnetic material according to the present invention is characterized, as compared with that consisting of Co-Fe-Nb, by exhibiting a high coercive force not less than 35 Oe, preferably from 40 to 70 Oe, more preferably from 60 to 70 Oe, a residual magnetization flux density of not less than 11 kG preferably 13 kG, and a fullness factor of not less than approximately 0.80. In addition the energy product (BH)ₘₐₓ ranges advantageously from 0.3 to 0.6 M G.Oe.

A measurement of the resistivity and an X-ray diffractometry was carried out with regard to the alloy materials of Co-15%Fe-4%Nb-2-5%Mo, which were firstly formed in the form of a coil having a 2 mm diameter and, then, drawn to a size of 0.6 mm after being solution treated at 1100°C. The drawn coil was subjected to ageing at a temperature up to 1000°C and then, resistivity measurement and X-ray diffractometry were carried out. The results of such measurement and X-ray diffractometry are shown in Fig. 1.

The following facts will be apparent from Fig. 1. (1) The decrease of resistivity starts from 500°C. (2) The resistivity is minimum at a temperature of from 650 to 700°C. (3) The resistivity is increased from a temperature higher than 700°C. (4) The alloy materials exhibit at a drawing state (A.D.) a crystal structure of a face centered cubic (FCC) lattice with a lattice constant (a) of 3.56 angstroms. (5) The face centered cubic phases of the alloy material at the drawing state are decomposed into the new phases of the body centered cubic (BCC) lattice and precipitates (PPT), as well as the original face centered cubic (FCC) phases, while the resistivity is decreased during the decomposition. (6) Only the face centered cubic (FCC) phases are present at a temperature of 800°C and higher.

It was proven by the X-ray diffractometry of the alloy materials that the face centered cubic phases and the body centered cubic phases are a solid solution of cobalt, and the iron is dissolved in the solid solution. The composition of the precipitated phases are not elucidated but are believed to be the intermetallic compounds of Co₃Nb and Co₃Mo.

From the facts revealed from Fig. 1, it will be apparent that several features of the present invention reside in the structure of the alloy materials. The increase of coercive force by ageing at a temperature of from 600 to 750°C is caused not only by a precipitation of the intermetallic compounds into the cobalt matrix, as in the case of the known, Co-Fe-Nb alloy, but also by a decomposition of the cobalt matrix into the FCC phases and BCC phases. Such decomposition of the cobalt matrix into two kinds of phases is believed to cause the remarkabie increase of the coercive force, which increase is achieved when the molybdenum is added in an amount of at least 2%. When the matrix of any metallic material is composed of the two kinds of mixture phases, the cold workability thereof is impaired thereby. In addition, the decomposition of the matrix is liable to occur even during the cold drawing in the case of the known Co-Fe-Nb alloy material. However, according to one of the features of the invention, the cobalt matrix is not decomposed due to the Mo addition during the cold working, and thus the cold workability of the alloy materials is not impaired advantageously.

In Fig. 2, the hardness after drawing is shown with regard to the several cobalt-based alloys. The lines -0- and -0- represent the alloy of Co-15%Fe-2%Nb-x%Mo and the alloy of Co-15%Fe-4°/Nb-x%Mo, according to the present invention, respectively. The line ―⊙― represents the alloy of Co-12%Fe-x%Ti, the line represents the alloy of Co-12%Fe- x%Nb, and the line -0- represents the alloy of Co-11%Fe-5%Ti-x%Mo. All the alloys were cold drawn at a reduction of area of 90%. From Fig. 2, the influence of the additional element, i.e. molybdenum, niobium or titanium, on the work hardening of Co-Fe alloys is apparent. The molybdenum content exerts substantially no influence on the hardness of the Co-Fe alloy materials (c.f. the lines ―Δ―, -0-and ―⊙―). In the alloys represented by these three lines, the alloy of Co-1 1%Fe-5%Ti-x%Mo has the highest hardness, while the other two alloys have an advantageously low hardness of not exceeding 450 in Vickers. When the titanium- or niobium-content is increased, the hardness is also proportionally increased (the line ―⊙― or ―⊙).

In Table I, below, the cold workability, the coercive force (Hc in Oe) and the saturation flux density (Bᵢₒₒ in kG) are shown with regard to the known, Co-Fe-Nb alloys disclosed in U.S. Patent No. 3,989,557. These alloys were produced using the same procedure as in Example 1, illustrated hereinbelow. Since the difficulty in the workability cannot be quantitatively expressed, it is expressed in the three levels A, B and C, wherein the level A indicates that the alloy material could be worked into a wire having diameter of 0.6 mm (reduction of area of 91 %), the level B indicates that the wire was frequently ruptured during the drawing to the size of 0.6 mm, and the level C indicates that the 0.6 mm wire could not be produced by the drawing. The magnetic properties in Table I are those of the wires having a diameter of 0.6 mm and aged at 700°C. However, with regard to the wires of level C, the magnetic properties of the actually produced wires were measured and then calibrated, in a manner as if the change of the magnetic properties occurred due to the cold drawing of the wires up to 91% of the reduction of area.

It is apparent from Table I, that the cold workability of the alloy materials exhibiting a coercive force more than 36 Oe is B or C. The cold workability is deteriorated with an increase in the niobium and iron contents. Although either the high coercive force or the excellent cold workability must be sacrificed in the known alloy materials consisting of cobalt, iron and niobium, both the required, coercive force and cold workability can be achieved by the addition of molybdenum to this alloy material. According to one of the features of the present invention, the rupture of the wire during the cold drawing is considerably decreased in the present invention as compared with that in the cold drawing of the known alloy material of Co-Fe-Nb. The alloy material according to the present invention can be drawn at a reduction of area of at least 90% without the wire rupturing. Although the wire according to the known alloy of Co-Fe-Nb is broken into more than three pieces, the wire according to the present invention is not broken during drawing, even if both wires are drawn under the same drawing conditions.

The hardness after cold drawing is the result of the work hardening and is a factor which influences the cold workability of any metallic material. The relationship between the cold workability and the coercive force of the cobalt based alloy materials is readily seen in Fig. 3. In Fig. 3, the line --α- represents the known alloy material of Co-12%Fe-x%Nb, which is cold drawn at a reduction of area of 90% (except for 65% of the alloy containing 6%Nb) and which is aged at 700°C for the period of 1 hour. The alloy material is Co-12%Fe-6%Nb could not be cold drawn at a reduction of area of 90%. The line ―○― represents the alloys materials according to the present invention, which consists of Co-1 5%Fe-4%Nb-x%Mo. These alloy materials were drawn at a reduction of area of 90% and the hardness of the alloy materials after the cold drawing was measured. The cold drawn alloy materials were then aged at 650°C for the period of 1 hour. The known alloy materials exhibit the increase of coercive force with an increase in the hardness after drawing, i.e. a deterioration of the cold workability. In other words, due to the precipitation of intermetallic compounds containing niobium, the coercive force is increased, while the intermetallic compounds containing niobium, which are left undissolved in the cobalt matrix, reduce or impair the cold workability of the known alloy of Co-Fe-Nb. On the other hand, in the alloy materials according to the present invention, the coercive force is advantageously increased from 35 to 75 Oe, while the hardness after drawing is kept essentially constant. This fact means that the amount of the intermetallic compounds, which are supposed to contain molybdenum, in addition to niobium, is not changed regardless of the increase of the coercive force. The difference between the two lines in Fig. 3 implies, therefore, that in the alloy materials of the present invention, the increased coercive force in the range from 35 to 70 Oe is caused mainly due to the decomposition of the cobalt matrix into the new body centered cubic (BCC) phases and the original face centered cubic (FCC) phases, explained in connection with Fig. 1. In other words, the precipitation of the intermetallic compounds does not act a major role to such increase of the coercive force.

Referring to Fig. 4 a coil form 1 contains a plurality of reed switches which are used as crosspoint switches, and outside of each 1, a driving coil 8, which is connected to a conductor 5 and drives the above-mentioned reed switch, is wound. A magnetic shunt plate 2 is composed of magnetic material and provides a plurality of holes for arranging the above-mentioned coil forms 1 in matrix array. Horizontal and vertical multiple connecting wires 3, 4 and 9 shown in Fig. 5, connect the lead terminals 6 of the reed switches held in the coil forms 1 with the output terminals of the circuits of the speech path. Said multiple connecting wires 3, 4 and 9 are composed of high permeability magnetic material and are capable of relieving the prominent demagnetizing effect between reed switches. Such demagnetizing phenomenon is frequently produced when the reed switch is miniaturized.

As shown in Fig. 5, four reed switches are inserted in the respective coil forms 1 so as not to lie on the same line with respect to the longitudinal directions of the respective multiple connecting wires 3 and 9, and connected to said respective multiple connecting wires 3 and 9. Thus, the multiple connecting wires 3 and 9 are respectively arranged on the same plane in parallel, with a substantially equal distance between adjacent connecting lines. Fig. 6 shows the relation between the coil form 1 and the reed switches 13-15 which are contained in the coil form 1. Referring to Fig. 6, four reed switches 13, 14, 15 and 16 are contained in the coil form 1, and the lead ends 6 of these reed switches are arranged in row and column direction as shown in Figure 5, and connected with the multiple connection wires.

In the crosspoint switches as shown in Figs. 4, 5 and 6, the hysteresis loop of the semi-hard magnetic materials of the reed switches are distorted by the mutual demagnetization effect, in such a manner that the energy product (BH)ₘₐₓ of the hysteresis loop is decreased. However, since the semi-hard magnetic material according to the present invention exhibits a high coercive force, it is advantageously used for the reed pieces of reed switches of a four wire crosspoint switching matrix.

The present invention is explained more in detail in connection with Examples.

### Example 1

Electrolytic cobalt, electrolytic iron, ferro- niobium metal and ferromolybdenum metal were charged in an aluminous crucible and melted under vacuum by a high frequency induction furnace. The obtained melt was cast to produce an ingot having a diameter of 4Q mm and a weight of approximately 3.2 kg. The ingot was homogenized at 1200°C for 5 hours and subsequently worked to a wire of 2 mm in diameter by using a hot swaging machine, cold swaging machine and a wire drawing machine. This wire of 2 mm in diameter was heated at 1100°C for 30 to 60 minutes to carry out the solution treatment, and directly after the heating quenched in water. The so treated wire of 2.0 mm in diameter was cold drawn to the size of 0.6 mm in diameter, and the reduction of area during the cold drawing amounted to 91 %. The wire could be cold drawn without occurrence of rupturing. The cold workability was excellent. The cold drawn wire was subjected to an ageing at a temperature of from 600° to 750°C for one hour. The so produced semi-hard magnetic material contained 15% of iron 4% of niobium, from 2 to 5% of molybdenum and cobalt in the balance.

The measurement results of coercive force (Hc), the residual flux density (Br), and the squareness ratio (Br/Bs, Bs designates the saturation flux density) are shown in Figs. 7A, B and C.

The following facts will be apparent from Figs. 7A, B and C. When the aging temperature is adjusted from 600 to 700°C, preferably from 630 to 660°C, (1) the coercive force is 40 Oe or more, preferably from 50 Oe or more, (2) the squareness ratio ranges from 92 to 95%, and (3) residual magnetization ranges from 11 to 14 kG. Accordingly, several properties required for the semi-hard magnetic materials are satisfied by adjusting the ageing temperature. The molybdenum content should be not more than 5%, so as to provide the semi-hard magnetic material with high residual flux density.

The residual flux density and coercive force measured in the present Example are shown in Figs. 8A and B, respectively, in dependence upon the molybdenum content. As is clear from Fig. 8B, the increase of the coercive force with the increase of molybdenum content is ten or more times larger at the molybdenum content of 2% or more than at the molybdenum content of less than 2%. This fact well coincides with the difference in the crystallographic structure of the aged Co-Fe alloy materials, between the alloy materials containing 2% or more of molybdenum and those containing no molybdenum. Such difference is explained in detail in connection with Fig. 1. It can therefore be believed that the crystallographic change of the alloy materials containing less than 2% of molybdenum is similar to that of the known, Co-Fe-Nb alloy.

### Example 2

The cobalt-based, semi-hard magnetic material containing 18% of iron, 3% of niobium and from 2 to 5% of molybdenum was produced by the procedure of Example 1.

In Figs. 9A, B and C similar to Figs. 7A, B and C, respectively, almost same measured results of the coercive force, residual flux density and squareness ratio as in those of Figs. 7A, B and C, respectively, are obtained, except for the following. The coercive force and residual flux density :n Figs. 9A and B, respectively are slightly higher than in those of Figs. 7A and B. The squareness ratio in Fig. 9C.

The influence of molybdenum on the residual flux density and coercive force as seen from Figs. 10A and B, respectively, is different from that as seen from Figs. 8A and B in the following points. In Fig. 10A, the decrease of the residual flux density with the increase of the molybdenum content is advantageously mitigated. In FIG. 10B, the coercive force of the aged alloy materials is higher than that of the aged alloy materials in Fig. 8B containing the same amount as in Fig. 10B. These differences are advantageous from the point of view of magnetic properties, and are caused by lower niobium and higher iron content of the alloy materials in Fig. 10 than in those in Fig. 8.

### Example 3

The cobalt-based, semi-hard magnetic material containing from 12 to 18% of iron, 4% of niobium and 3% of molybdenum was produced by the procedure of Example 1.

Figs. 11A, B and C are graphs similar to Figs. 7A, B and C, respectively.

When the alloy materials containing 18% and 15% of iron are compared with the alloy material containing 12%, of iron, the latter exhibits the inferior, coercive force and squareness ratio to those of the former. The iron content is therefore preferably not less than 15%, from the point of view of magnetic properties.

It is clear from Fig. 12, that although the coercive force proportionally increases with the iron content, the residual magnetization is left almost unchanged.

The squareness ratio of the alloy materials produced in the present Example ranged from 90 to 95%.

### Example 4

The semi-hard magnetic materials having three compositions as shown in Table 11 were produced by the procedure of Example 1. The measurement results of the magnetic properties are illustrated in Table II.

## Claims

1. A magnetic material for a reed pice of a reed switch, said material containing (a) cobalt and iron, which forms a matrix of said material having a face centred cubic lattice, (b) additional niobium, which niobium is precipitated in said matrix as intermetallic compounds and provides said material with the required coercive force, and (c) one element, which is added in a predetermined amount, characterised in that said one element is molybdenum and is present in said material in an amount of not less than 2% by weight so that said matrix is composed of said face centred cubic lattice and a body centred cubic lattice, said material has a coercive force of not less than 35 Oe, preferably from 40 to 70 Oe, more preferably from 60 to 70 Oe, and the components of said material are present in the following ranges by weight:
iron from 12 to 18%, preferably from 15 to 18%;
niobium from 2 to 4%;
molybdenum from 2 to 5%;
and the balance essentially cobalt, thereby providing said material with a residual magnetization flux density of not less than 11 kG, preferably 13 kG, and a fullness factor of not less than approximately 0.80, the fullness factor being represented by the formula: wherein (BH) max is the maximum magnetic energy product and Hc is coercive force.

2. A process for producing a reed piece of a reed switch from a magnetic material containing cobalt and iron, and additionally niobium and one element which is added in a predetermined amount, the process comprising the steps of solution-treating said material, cold working said solution-treated material at a predetermined reduction area, ageing said cold worked material, and enclosing said aged material in a glass capsule of said reed switch, characterised in that molybdenum is selected as said one element in an amount of from 2 to 5% by weight and the iron content is adjusted to an amount in the range of from 12 to 18%, preferably from 15 to 18%, by weight, and the niobium content to an amount in the range of from 2 to 4% by weight, said cold working is performed at a reduction of area of at least 90%, and, due to said molybdenum selection, (a) maintaining the hardness of said cold worked material at a value not exceeding 450 Vickers Pyramid Number, (b) preventing the decomposition of the cobalt matrix phases of the face centred cubic lattice into two different kinds of phases during said cold working, and (c) preventing the rupture of said material during said cold working; said cold worked material is aged at a temperature of from 600 to 750°C, preferably from 650 to 700°C thereby decomposing said cobalt matrix phases into (a) the phases of intermetallic compounds precipitated in the matrix of said aged material, (b) the original matrix phases of said face centred cubic lattice and (c) the new matrix phases of a body centred cubic lattice; and the magnetic alloy is provided with a coercive force not less than 35 Oe, preferably from 40 to 70 Oe, more preferably from 60 to 70 Oe, a residual magnetisation flux density of not less than 11 kG, preferably 13 kG, and a fullness factor of not less than approximately 0.80, the fullness factor being represented by the formula: wherein (BH)max is the maximum magnetic energy product and Hc is coercive force.

3. A process according to Claim 2, characterised in that said solution treatment is performed at a temperature of from 1050 to 1200°C, preferably from 1050 to 1150°C.

4. A process according to Claim 2 or Claim 3, characterised in that said process further comprises applying a metallic coating layer to said aged material.

5. The use of a reed piece of a semi-hard magnetic material according to Claim 1, for a four wire crosspoint switch.

## Revendications

1. Matériau magnétique pour lame d'interrupteur, ledit matériau étant du type qui contient (a) du cobalt et du fer formant une phase continue ayant un réseau cristallin cubique à faces centrées, (b) une quantité supplémentaire de niobium qui précipite dans la phase continue sous forme de composés intermétalliques et donne au matériau le champ coercitif nécessaire, et (c) un élément qui est ajouté en quantité prédéterminée, ledit matériau étant caractérisé en ce que ledit élément ajouté en quantité prédéterminée est le molybdène et est présent dans la matériau en quantité au moins égale à 2% en poids afin que la phase continue soit formée du réseau cubique à faces centrées et d'un réseau cubique centré, le matériau ayant un champ coercitif qui n'est pas inférieur à 2900 A/m et qui est de préférence compris entre 3200 et 5600 A/m, très avantageusement entre 4800 et 5600 A/m, et les éléments constituants du matériau sont présents dans les plages pondérales suivantes:
12 à 18% et de préférence 15 à 18% de fer,
2 à 4% de niobium,
2 à 5% de molybdène,
et le reste pratiquement de cobalt, si bien que le matériau a une densité de flux d'aimantation résiduelle qui n'est pas inférieure à 1,1 T et qui est de préférence de 1,3 T, et un facteur d'occupation qui n'est pas inférieur à 0,80 environ, le facteur d'occupation étant représenté par la formule dans laquelle (BH)max représente le produit du champ par l'induction correspondant à l'énergie maximale et Hc représente le champ coercitif.

2. Procédé de fabrication d'une lame d'interrupteur à partir d'un matériau magnétique contenant du cobalt et du fer avec en plus du niobium et un élément qui est ajouté en quantité prédéterminée, le procédé étant du type qui comprend un recuit de mise en solution du matériau, l'écrouissage du matériau traité correspondant à une striction prédéterminée, le vieillissement du matériau écroui, et l'enrobage du matériau vieilli dans une capsule de verre de l'interrupteur à lame, ledit procédé étant caractérisé en ce que ledit élément est le molybdène présent en quantité comprise entre 2 et 5% en poids, et la teneur en fer est réglée à une valeur comprise entre environ 12 et 18% et de préférence entre environ 15 et 18% en poids, et la teneur en niobium est réglée à une valeur comprise entre 2 et 4% en poids, l'écrouissage étant effectué de manière qu'il corresponde à une striction d'au moins 90% et, du fait de la sélection du molybdène, assurant (a) le maintien de la dureté de la matière écrouie à une valeur ne dépassant pas l'indice de dureté Vickers 450 mesuré à la pyramide, (b) l'inhibi- tion de la décomposition des phases continues de cobalt du réseau cubique à faces centrées en deux types différents de phases pendant l'écrouissage, et (c) l'inhibition de la rupture du matériau pentant l'écrouissage, le matériau écroui subissant un vieillissement à une température comprise entre 600 et 750⁰C et de préférence entre 650 et 700°C afin que les phases continues de cobalt se décomposent en (a) phases de composés intermétalliques précipités dans la phase continue du matériau vieilli, (b) phase continue originale du réseau cubique à faces centrées et (c) nouvelles phases continues d'un réseau cubique centré, et l'alliage magnétique a un champ coercitif qui n'est pas inférieur à 2900 A/m, de préférence compris entre 3200 et 5600 A/m, et très avantageusement compris entre 4800 et 5600 A/m, une densité de flux d'aimantation résiduelle qui n'est pas inférieure à 1,1 T et de préférence 1,3 T, et un facteur d'occupation qui n'est pas inférieur à 0,80 environ, ce facteur d'occupation étant représenté par la formule dans laquelle (BH)max désigne le produit du champ et de l'induction magnétiques correspondant à l'énergie maximale et Hc désigne le champ coercitif.

3. Procédé selon la revendication 2, caractérisé en ce que le recuit de mise en solution est effectué à une température comprise entre 1050 et 1200°C, de préférence entre 1050 et 1150°C.

4. Procédé selon l'une des revendications 2 et 3, caractérisé en ce qu'il comporte en outre l'application d'une couche métallique de revêtement sur le matériau vieilli.

5. Application du matériau magnétique selon la revendication 1, ayant une perméabilité magnétique moyennement élevée, à une lame d'interrupteur pour points de croisement à quatre fils.

## Patentansprüche

1. Magnetisches Material für ein Zungenstück eines Reed-Schalters, das (a) Kobalt und Eisen, was eine Grundmasse dieses Materials mit einem flächenzentrierten kubischen Gitter bildet, (b) zusätzlich Niobium, das in der Grundmasse als intermetallische Verbindung abgeschieden ist und dem Material die erforderliche Koerzitivkraft gibt, und (c) ein Element, das in einer vorbestimmten Menge hinzugefügt wird, enthält, dadurch gekennzeichnet, daß das eine E!ement Molybdän und in dem Material in einer Menge von nicht weniger als 2 Gew.-% vorhanden ist, so daß die Grundmasse aus dem genannten flächenzentrierten kubischen Gitter und einem raumzentrierten kubischen Gitter zusammengesetzt ist, das Material eine Koerzitivkraft von nicht weniger als 35 Oe, vorzugsweise von 40 bis 70 Oe, mit besonderem Vorteil von 60 bis 70 Oe, besitzt und die Komponenten des Materials in den folgenden Gewichtsbereichen vorliegen:
Eisen von 12 bis 18%, vorzugsweise von 15 bis 18%;
Niobium von 2 bis 4%;
Molybdän von 2 bis 5%;
und der Rest im wesentlichen Kobalt, wodurch das Material mit einer magnetischen Restflußdichte von nicht weniger als 11 kG, vorzugsweise 13 kG, und einem Füllfaktor von nicht weniger als etwa 0,80 versehen wird, wobei der Füllfaktor durch die Formel dargestellt wird: wobei (BH)max das maximale magnetische Energieprodukt und Hc die Koerzitivkraft ist.

2. Verfahren zur Herstellung eines Zungenstücks eines Reed-Schalters aus einem magnetischen Material, das Kobalt und Eisen und zusätzlich Niobium und ein Element enthält, das in einer vorbestimmten Menge hinzugefügt ist, wobei das Verfahren die Schritte des Lösungsglühens des Materials, des Kaltverformens des lösungsgeglühten Materials auf eine vorbestimmte Querschnittsverminderung, das Altern des kaltverformten Materials und das Einschließen des gealterten Materials in eine Glashülle des Reed-Schalters umfaßt, dadurch gekennzeichnet, daß als das eine Element Molybdän in einer Menge von 2 bis 5 Gew.-% ausgewählt und der Eisenanteil auf eine Menge im Bereich von 12 bis 18 Gew.-%, vorzugsweise 15 bis 18 Gew.-%, und der Niobiumgehalt auf eine Menge im Bereich von 2 bis 4 Gew.-% eingestellt wird, wobei die Kaltverformung auf eine Querschnittsverminderung von wenigstens 90% durchgeführt und wegen der Molybdänwahl (a) die Vickers-Härte des kaltverformten Materials auf einem nicht über 450 liegenden Wert gehalten, (b) die Zerlegung der Phasen mit flächenzentriertem kubischen Gitter der Kobalt-Grundmasse in zwei verschiedene Arten der Phasen während der Kaltverformung verhindert und (c) das Reißen des Materials während der Kaltverformung verhindert wird, wobei des kaltverformte Material bei einer Temperatur von 600 bis 750°C, vorzugsweise von 650 bis 700°C, gealtert wird, wodurch die Phasen der Kobalt-Grundmasse zerlegt werden in (a) die Phasen der in der Grundmasse des gealterten Materials abgeschiedenen intermetallischen Verbindungen, (b) die ursprünglichen Phasen der Grundmasse mit flächenzentriertem kubischem Gitter und (c) die neuen Phasen der Grundmasse mit einem raumzentrierten kubischen Gitter, und wobei die magnetische Legierung mit einer Koerzitivkraft von nicht weniger als 35 Oe, vorzugsweise von - 40 bis 70 Oe, mit besonderem Vorteil von 60 bis 70 Oe, einer magnetischen Restflußdichte von nicht weniger als 11 kG, vorzugsweise 13 kG, und einem Füllfaktor von nicht weniger als 0,80 versehen wird, wobei der Füllfaktor durch die Formel: dargestellt ist, in der (BH)max das maximale magnetische Energieprodukt und Hc die Koerzitivkraft ist.

3. Verfahren nach Anspruch 2, dadurch gekennzeichnet, daß das Lösungsglühen bei einer Temperatur von 1050 bis 1200°C, vorzugsweise von 1050 bis 1150°C, durchgeführt wird.

4. Verfahren nach Anspruch 2 oder 3, dadurch gekennzeichnet, daß das Verfahren ferner das Aufbringen einer metallischen Uberzugsschicht auf dem gealterten Material umfaßt.

5. Verwendung eines Zungenstücks eines halbharten Magnetmaterials gemäß Anspruch 1 für einen vieradrigen Kreuzpunktschalter.
